

## UNITED STATES PATENT OFFICE

2,603,638

PRODUCTION OF ORGANIC ACID ESTERS  
OF CELLULOSE

George W. Seymour, Maplewood, Blanche B. White, Summit, and Mark Plunguian, Gillette, N. J., assignors to Celanese Corporation of America, New York, N. Y., a corporation of Delaware

No Drawing. Application December 22, 1950,  
Serial No. 202,406

7 Claims. (Cl. 260—229)

1

This invention relates to the production of organic acid esters of cellulose and relates more particularly to an improved process for the production of organic acid esters of cellulose which may be carried out in a continuous manner.

This application is a continuation-in-part of application S. No. 115,946, filed September 15, 1949.

In the production of organic acid esters of cellulose by the esterification of a cellulosic material, it is customary to pretreat the cellulosic material before esterification to increase its reactivity and thereby reduce the total esterification time. To enable the production of the organic acid esters of cellulose to be carried out in a continuous manner, the pretreatment should require only a relatively short period of time. In addition, the pretreatment should increase the reactivity of the cellulosic material to a point where the esterification thereof will be completed rapidly.

It is an important object of this invention to provide a process for the production of organic acid esters of cellulose which will fulfill the foregoing requirements and which may be carried out in a continuous manner.

A further object of this invention is to provide a novel process for pretreating cellulosic material which may be carried out in a relatively short period of time and which will render said cellulosic material highly reactive.

Other objects of this invention will be apparent from the following detailed description and claims.

In accordance with the present invention, cellulosic material is subjected to a two-stage pretreatment prior to esterification. During the first stage of the pretreatment, the cellulosic material has added thereto a lower aliphatic acid in the presence of from about 4 to 9 parts by weight of water, or preferably from about 4 to 7 parts by weight of water for each 100 parts by weight of the cellulosic material. After all the treating agents have been added to the cellulosic material for the first stage of the pretreatment, an interval of at least about 2 minutes, or preferably at least about 3 minutes, is permitted to elapse. Then, the cellulosic material has added thereto, during the second stage of the pretreatment, which does not exceed about 15 minutes, an additional quantity of a lower aliphatic acid containing from about 3 to 15 parts by weight of an esterification catalyst for each 100 parts by weight of the cellulosic material.

The process of the present invention may be applied to any suitable cellulosic material, such

as cotton linters, or wood pulps or the like from which the lignin, pentosan, resins and similar constituents have been removed, as, for example, purified sulfite pulp, sulfate pulp or soda pulp.

5 In addition, there may be employed cellulosic material derived from other sources such as bamboo, reeds, jute, esparto, straws such as linseed and hempseed straw, grasses, peanut hulls, bark, etc. The cellulosic material may be pretreated in the form of a mass of loose fibers, or in the form of a sheet, strip or board. The term "cellulosic material" as employed herein is to be construed as meaning cellulose which may contain smaller quantities of other substances such as the residual impurities that remain therein following the purification processes referred to above.

Any of the lower aliphatic acids including formic, acetic, propionic and butyric acids, as 20 well as mixtures thereof, may be employed during the first stage of the pretreatment in amounts of from about 15 to 75 parts by weight or preferably from about 30 to 40 parts by weight for each 100 parts by weight of the cellulosic material. There 25 must also be present during the first stage of the pretreatment, from about 4 to 9 parts by weight of water for each 100 parts by weight of the cellulosic material. The necessary amount of water may be present in or may be added to the 30 cellulosic material before the pretreatment begins, or it may be included in the lower aliphatic acid employed for the pretreatment, or a portion of the water may be present in or added to the cellulosic material before the pretreatment begins and the remainder of the water may be included in the lower aliphatic acid.

The temperature employed during the first stage of the pretreatment is not critical and may range from about 25 to 55° C. To obtain a cellulosic material having the highest reactivity, a 40 short interval of time should be permitted to elapse after all the treating agents have been added to the cellulosic materials for the first stage of the pretreatment and before the second stage 45 of the pretreatment is begun. At temperatures of up to about 35° C., this interval should be at least about 3 minutes. At higher temperatures, an interval of at least about 2 minutes will be adequate.

50 The first stage of the pretreatment is followed, in the second stage of the pretreatment, by the treatment of the cellulosic material, for a period not exceeding about 15 minutes and preferably between about 2 and 5 minutes, with an additional quantity of a lower aliphatic acid contain-

ing from about 3 to 15 parts by weight of an esterification catalyst for each 100 parts by weight of the cellulosic material. The lower aliphatic acid is preferably employed, during the second stage of the pretreatment, in amounts of from about 100 to 600 parts by weight or preferably from about 150 to 300 parts by weight for each 100 parts by weight of the cellulosic material.

Any of the known acid cellulose esterification catalysts may be employed for pretreating the cellulosic material in accordance with the process of this invention, but it is preferred to employ sulfuric acid for this purpose since it produces a cellulosic material having the highest reactivity in the shortest period of time.

The pretreating agents may be applied to the cellulosic material in any desired manner. For example, they may be sprayed or rolled onto the cellulosic material, or, when the cellulosic material is in the form of a sheet, strip or board, the pretreating agents may be applied as a continuous film from a perforated or slotted conduit extending the width of the sheet, strip or board.

The pretreated cellulosic material is esterified with an organic acid anhydride, which may contain additional quantities of lower aliphatic acid and esterification catalyst. Esterification proceeds rapidly and is completed in about 15 to 30 minutes, or less. The lower aliphatic acid acts as a solvent for the cellulose ester so that the product is obtained in the form of a clear dope. After the esterification is complete, a sufficient quantity of water is added to the esterification mixture to convert any remaining organic acid anhydride to the corresponding acid, following which the cellulose ester, preferably after the addition of a further quantity of water, is permitted to hydrolyze or ripen to impart the desired solubility characteristics thereto. The cellulose ester is then precipitated from the esterification mixture, washed to free it from acids and other impurities, stabilized if necessary, washed again and finally dried. When the process of this invention is employed for the preparation of organic acid esters of cellulose, it is possible to carry out both the pretreatment and esterification on a continuous rather than on a batch basis, since the time required for both steps is sufficiently short to render a continuous process feasible.

Our invention will now be described specifically in connection with the production of cellulose acetate, which is commercially the most important organic acid ester of cellulose at the present time. It may, however, also be employed for the production of other organic acid esters of cellulose such as, for example, cellulose propionate, cellulose butyrate, cellulose acetate propionate and cellulose acetate butyrate.

The following examples are given to illustrate this invention further.

#### Example I

Onto 100 parts by weight of cotton linters containing 6 parts by weight of water, there is sprayed 35 parts by weight of acetic acid and the cotton linters are stirred for 5 minutes. The cotton linters are then sprayed with 300 parts by weight of acetic acid containing 15 parts by weight of sulfuric acid. After an interval of 4 minutes, the pretreated cotton linters are esterified by treatment with 220 parts by weight of acetic anhydride at a temperature of 35° C. Esterification is complete in 15 minutes as evidenced by the clearing of the esterification mixture.

#### Example II

Cotton linters are pretreated and esterified in the manner set forth in Example I, employing 10 parts by weight of sulfuric acid during the second stage of the pretreatment and adding 5 parts by weight of sulfuric acid to the acetic anhydride employed for the esterification of the pretreated cellulosic material. Esterification is complete in 15 minutes as evidenced by the clearing of the esterification mixture.

#### Example III

Cotton linters are pretreated and esterified in the manner set forth in Example I, employing 3 parts by weight of sulfuric acid during the second stage of the pretreatment and adding 12 parts by weight of sulfuric acid to the acetic anhydride employed for the esterification of the pretreated cellulosic material. Esterification is complete in 16 minutes as evidenced by the clearing of the esterification mixture.

When the quantity of sulfuric acid employed during the second stage of the pretreatment is reduced below about 3 parts by weight per 100 parts by weight of cellulosic material, the time required for esterification increases rapidly and, in many cases, the esterification does not go to completion.

#### Example IV

Onto 100 parts by weight of cotton linters that have been dried for 2 hours at 100° C. and contain 0.3 parts by weight of water, there is sprayed 35 parts by weight of acetic acid containing 6 parts by weight of water and the cotton linters are permitted to stand for 3 minutes. The cotton linters are then sprayed with 300 parts by weight of acetic acid containing 15 parts by weight of sulfuric acid. After an interval of 1 minute, the pretreated cotton linters are esterified by treatment with 220 parts by weight of acetic anhydride at a temperature of 35° C. Esterification is complete in 15 minutes.

If the water is omitted from the acetic acid employed during the first stage of the pretreatment, the esterification does not go to completion.

It is to be understood that the foregoing detailed description is given merely by way of illustration and that many variations may be made therein without departing from the spirit of our invention.

Having described our invention, what we desire to secure by Letters Patent is:

1. In a process for the preparation of organic acid esters of cellulose from cellulosic material, the steps which comprise subjecting the cellulosic material to a multi-stage pretreatment prior to esterification, one stage of said pretreatment comprising the addition to the cellulosic material of a lower aliphatic acid in the presence of from about 4 to 9 parts by weight of water for each 100 parts by weight of the cellulosic material, and another stage of said pretreatment comprising the addition to the cellulosic material of a lower aliphatic acid containing from about 3 to 15 parts by weight of an esterification catalyst for each 100 parts by weight of cellulosic material without displacing any of the lower aliphatic acid contained in the cellulosic material, and esterifying the pretreated cellulosic material within a period of less than about 15 minutes after the addition thereto of the lower aliphatic acid and the esterification catalyst.
2. Process according to claim 1, wherein from about 15 to 75 parts by weight of lower aliphatic

acid for each 100 parts by weight of cellulosic material are employed during the initial stage of the pretreatment, and from about 100 to 600 parts by weight of lower aliphatic acid for each 100 parts by weight of cellulosic material are employed during the second stage of the pretreatment.

3. Process according to claim 2, wherein there is an interval of at least about 2 minutes between the two stages of the pretreatment, and wherein acetic acid is employed as the pretreating acid and sulfuric acid is employed as the esterification catalyst.

4. In a process for the preparation of cellulose acetate from cellulosic material, the steps which comprise subjecting the cellulosic material to a multi-stage pretreatment prior to esterification, one stage of said pretreatment comprising the addition to the cellulosic material of a lower aliphatic acid in the presence of from about 4 to 9 parts by weight of water for each 100 parts by weight of the cellulosic material, and another stage of said pretreatment comprising the addition to the cellulosic material of a lower aliphatic acid containing from about 3 to 15 parts by weight of an esterification catalyst for each 100 parts by weight of cellulosic material without displacing any of the lower aliphatic acid contained in the cellulosic material, and acetylating the pretreated cellulosic material within a period of less than about 15 minutes after the addition thereto of the lower aliphatic acid and the esterification catalyst.

5. Process according to claim 4, wherein from about 15 to 75 parts by weight of lower aliphatic acid for each 100 parts by weight of cellulosic material are employed during the initial stage of the pretreatment, and from about 100 to 600 parts by weight of lower aliphatic acid for each 100 parts by weight of cellulosic material are employed during the second stage of the pretreatment.

6. Process according to claim 5 wherein there is an interval of at least about 2 minutes between the two stages of the pretreatment, and wherein acetic acid is employed as the pretreating acid

and sulfuric acid is employed as the esterification catalyst.

7. In a process for the preparation of cellulose acetate from cellulosic material, the steps which comprise subjecting the cellulosic material to a multi-stage pretreatment prior to esterification, one stage of said pretreatment comprising the addition to the cellulosic material of from about 30 to 40 parts by weight of acetic acid for each 100 parts by weight of cellulosic material in the presence of from about 4 to 7 parts by weight of water for each 100 parts by weight of cellulosic material, and another stage of said pretreatment comprising the addition to the cellulosic material after an interval of at least about 3 minutes of from about 150 to 300 parts by weight of acetic acid and from about 3 to 15 parts by weight of sulfuric acid for each 100 parts by weight of cellulosic material without displacing any of the acetic acid contained in the cellulosic material, and acetylating the pretreated cellulosic material within a period of less than about 15 minutes after the addition thereto of the acetic acid and sulfuric acid.

GEORGE W. SEYMOUR.

BLANCHE B. WHITE.

MARK PLUNGUIAN.

#### REFERENCES CITED

The following references are of record in the file of this patent:

#### UNITED STATES PATENTS

| Number    | Name           | Date          |
|-----------|----------------|---------------|
| 1,543,310 | Altwege        | June 23, 1925 |
| 2,028,761 | Dreyfus et al. | Jan. 28, 1936 |
| 2,063,324 | Malm et al.    | Dec. 8, 1936  |
| 2,113,301 | Gardner        | Apr. 5, 1938  |
| 2,122,572 | Jones et al.   | July 5, 1938  |
| 2,140,639 | Malm           | Dec. 20, 1938 |
| 2,206,288 | Malm           | July 2, 1940  |
| 2,315,973 | Malm           | Apr. 6, 1943  |
| 2,478,383 | Fordyce et al. | Aug. 9, 1949  |
| 2,478,425 | Richter et al. | Aug. 9, 1949  |
| 2,487,892 | Richter et al. | Nov. 15, 1949 |
| 2,552,190 | Lackey et al.  | May 8, 1951   |